

# UNITED STATES PATENT OFFICE.

MICHELE N. SALVATI, OF TURIN, ITALY; GUIDO BEER AND ARRIGO TEDESCO,  
EXECUTORS OF WILL OF SAID MICHELE N. SALVATI, DECEASED, ASSIGNORS  
TO SOCIETA ANONIMA STABILIMENTI BIAK, OF TURIN, ITALY.

## METHOD FOR COATING WITH TIN AND TIN ALLOYS ARTICLES MADE OF ALUMINIUM OR ALUMINIUM ALLOYS.

1,332,307.

Specification of Letters Patent.

Patented Mar. 2, 1920.

No Drawing.

Application filed November 15, 1918. Serial No. 262,708.

To all whom it may concern:

Be it known that I, MICHELE N. SALVATI, subject of the King of Italy, and resident of Turin, Italy, have invented certain new and useful Methods for Coating with Tin and Tin Alloys Articles Made of Aluminium and Aluminium Alloys, of which the following is a specification.

This invention has for its object a method by means of which a coating of tin and tin alloy may be applied on articles or parts made of aluminium or aluminium alloys, despite of the known property of aluminium that tin is unable to adhere thereto.

According to this invention, the surface of the article made of aluminium or aluminium alloy on which tin is to be applied, is previously coated with a layer of another metal capable of adhering firmly to aluminium and aluminium alloys without giving rise to an electrolytic action when in contact with aluminium, said coating metal being of such nature that tin and tin alloys adhere to it. As an example of said coating metals, copper, nickel, iron, zinc or the like may be mentioned.

Iron has in a particular manner said required character and the electrolytic process may be advantageously adopted for coating with it the aluminium and aluminium alloy surfaces on which tin is finally to be applied.

To this end the surface to be coated is firstly cleaned by means of a 10% solution of sodium hydrate and then is washed with water and is caused to act as a cathode into an electrolytic bath of an iron salt, by way of example into a solution of ferric sulfate; a proper quantity of ammonium oxalate may be advantageously added to said bath in order to increase homogeneity, cohesion and adherence of the iron layer or coating thus obtained.

As has been found by tests, satisfactory results are obtained by using an electrolytic bath comprising a mixture of equal portions of two solutions the first of them being formed of 40 grammes of ammonium oxalate dissolved into 1000 grammes of water and the other one consisting of 20 grammes of ferric sulfate dissolved into 1000 grammes of water; an electric current having a density of 0.15 ampere for each square decimeter of cathode may be conveniently used.

When an iron layer having the desired

thickness is obtained, the surface thereof is washed with water and dried with sawdust; thereafter tin or tin alloy may be applied on said surface by any desired method, a very satisfactory adherence being thus obtained.

What I claim as my invention and desire to secure by United States Letters Patent is:

1. A method for coating with tin and tin alloys articles made of aluminium and aluminium alloys, consisting in coating said aluminium article with an iron layer by electrolytic method, and then applying tin or tin alloy on said iron coating.

2. A method for coating with tin and tin alloys articles made of aluminium and aluminium alloys, consisting in treating said aluminium article in an electrolytic bath of ferric sulfate to coat it with an iron layer, and then applying tin or tin alloy on said layer.

3. A method for coating with tin and tin alloys articles made of aluminium and aluminium alloys, consisting in placing said aluminium article in a bath comprising equal amounts of a 4 per cent. solution of ferric sulfate and of a 2 per cent. solution of ammonium oxalate, connecting said article with the negative terminal of a source of electric current having a strength of 0.15 ampere for each square decimeter of surface to be coated, placing in said solution an iron plate connected with the positive terminal of said source to cause said current to circulate through said bath and to obtain an electrolytic iron layer on said article, washing and drying said layer and applying tin or tin alloy thereon.

4. A method for coating with tin and tin alloys articles made of aluminium and aluminium alloys, consisting in placing said aluminium article in a solution of ferric sulfate and ammonium oxalate, connecting said article with the negative terminal of an electric current source, placing in said solution an iron plate connected with the positive terminal of said source to cause said current to circulate through said solution, and obtain an electrolytic iron layer on said article, washing and drying said layer and applying tin or tin alloy thereon.

Signed at Turin, Italy, this 17th day of October, A. D. 1918.

MICHELE N. SALVATI.